

# UNITED STATES PATENT OFFICE.

ROBERT ABBOTT HADFIELD, OF WESTMINSTER, ALEXANDER G. M. JACK, OF SHEFFIELD,  
AND ISAAC BERNARD MILNE, OF TOTLEY, ENGLAND.

## MANUFACTURE OF ARMOR-PIERCING PROJECTILES.

1,139,412.

Specification of Letters Patent.

Patented May 11, 1915.

No Drawing. Application filed August 19, 1913, Serial No. 785,466. Renewed October 6, 1914. Serial No. 865,393.

*To all whom it may concern:*

Be it known that we, ROBERT ABBOTT HADFIELD, knight, F. R. S., ALEXANDER GEORGE MCKENZIE JACK, and ISAAC BERNARD MILNE, respectively of 22 Carlton House Terrace, Westminster, Rockhills, Brincliffe, Sheffield, Yorkshire, and Cross Grove House, Totley, in the county of Derby, subjects of the King of Great Britain and Ireland, have invented Improvements in or Relating to the Manufacture of Armor-Piercing Projectiles, of which the following is a specification.

This invention has for its object to produce armor piercing projectiles, particularly of large diameters, say of twelve inches and upward, that shall be better adapted than heretofore to completely perforate thick hard faced armor plates without becoming broken up or broken to such an extent as to interfere with their subsequent desired action.

For this purpose an armor piercing shell according to the present invention is made of good steel, such as nickel chromium steel, and subsequently treated in such a manner that the head or ogival forward portion of the shell is of different degrees of hardness varying say from a ball hardness of from about 600 to 700 at the pointed front end portion or zone through successive rearward zones of about 500, 400 and 300 ball hardness, the zone having a ball hardness of about 400 terminating rearwardly just in front of the forward end of the cavity in the shell and the zone having a ball hardness of about 300 extending rearward for a short distance around the shell cavity, the remaining rearward portion of the shell having a ball hardness under 300. In the production of such a shell, made say of nickel chromium steel, the shell after being formed to shape, as by casting it solid and then, after suitably annealing it, pressing it to shape in a suitable press, is hardened by subjecting it to two separate treatments of which the first consists in heating the shell in a suitable furnace to a hardening temperature while protecting the point thereof from direct contact with the heating medium in a manner well understood, so that this shoulder portion of the projectile is raised to a higher temperature than the point and the point to a higher temperature than the base, then dipping the shell point downward to its

base end in a cooling medium for example oil, then raising it for a certain distance and holding it raised for a time, then raising it still farther to a suitable zone depth for a certain time and then lowering it again to the base end. The second treatment consists in heating the base portion of the shell to a suitable tempering temperature while its pointed end portion is immersed to a suitable depth in water, after which it is immersed or quenched outright in a cooling medium for example water. The temperatures to which the various parts of the shell are heated, the depths and durations of immersion and other details can be variously modified to suit different sizes of shells and the steel of which they are made. In some cases the shell may be subjected to a third treatment after the character of the first mentioned treatment.

According to one example, carried out with a twelve inch shell having a length of about thirty four inches and made of nickel chromium steel having the following approximate composition, namely carbon .6 to .7%; nickel 2 to 3% and chromium 2 to 3%, for example carbon about .66%, Ni about 2.52% and chromium about 2.31%, the shell was taper heated while its point was protected from direct contact with the heat, so that the external shoulder portion of the shell had a temperature of about 915° C. to 920° C. the inner surface or core adjacent to the shoulder portion a temperature of about 900 to 905° C., the point a temperature of about 890° C. and the base a temperature of about 780° C. The shell thus heated was then dipped in oil to its base end and held there for about eight minutes, then raised in the oil about twelve inches and held in that position for about ten minutes, then raised to a zone depth say of about ten inches and held in that position for about twenty five minutes, then lowered again to its base end and water poured into its interior. The shell was then subjected to a second treatment consisting in heating the base in a furnace to a temperature of about 670 to 705° C.; and its interior or core to a temperature of about 605° C. while its pointed end portion is immersed to a depth of about eight and a half inches in water kept cold. The shell was then allowed to cool down in the furnace

to a base temperature of about 320° C. to 300° C., and an internal or core temperature of about 290° C. to 255° C. whereupon the shell was quenched outright in water. 5 When thus treated, the pointed portion of the shell for about the first ten inches of its length had a ball hardness of 600 and over the weight of this portion comprising about 12% of the total weight of the projectile, 10 the ball hardness varying from 600 at ten inches from the point to 418 at fourteen inches, 311 at 18 inches and 241 at the base end of the shell, which had a length of about thirty four and a half inches.

15 According to another example carried out with a fourteen inch shell having a length of about fifty-two inches and made of nickel-chromium steel having the following approximate composition viz., carbon .69% nickel 2.53% and chromium 2.70%, the shell was taper heated while its point was protected from direct contact with the heat so that the external shoulder portion of the shell had a temperature of about 930° C., 20 the inner surface or core adjacent to the shoulder a temperature of about 900 to 905° C. the point a temperature of about 875° C. and the base a temperature of about 850° C. The shell thus heated was then dipped 25 in oil to its base end and held in that position for about 14 minutes, then raised in the oil about eighteen inches and held in that position for about four minutes then raised about six inches more and held for 30 about six minutes and then raised to a zone depth of about eleven inches and held there for eighteen minutes then lowered in the oil to its base end and about two gallons of water poured into its interior. The shell 35 was then subjected to a second treatment consisting in heating the base to a temperature of about 700° C. and its interior or core to a temperature of about 630 while its point is immersed for about a depth of 40 eight inches in water. The shell was then allowed to cool down in the furnace to a base temperature of about 310° C. and a core temperature of about 255° C. and then quenched outright in water. In this case 45 the first eight inches had a ball hardness of 652 and over this portion constituting about 6% of the weight of the shell, the hardness decreasing to the base where it is about 262.

50 From the foregoing examples it will be seen that the temperatures to which the various parts of the shell can be heated and the manipulation of the shell can be variously modified without departing from the essential features of the invention.

55 60 The above mentioned temperatures may be varied within a range of about 5% upward or downward.

What we claim is:—

1. The process of treating an armor pierc-

ing projectile which consists in heating the shell to a hardening temperature, to bring the shoulder to a higher temperature than the point and the point to a higher temperature than the base, then dipping the shell point downward to its base in a cooling 70 medium, maintaining it in that position for a few minutes, raising it about one third of its length more or less and there maintaining it for a few minutes, then raising to about two-thirds of its length more or 75 less and there maintaining for a somewhat longer time, then lowering in the medium to the base end and pouring water into its interior.

2. The process of treating an armor piercing projectile which consists in heating the shell to a hardening temperature, to bring the shoulder to a higher temperature than the point and the point to a higher temperature than the base, then dipping the shell 80 point downward to its base in oil, maintaining it in that position for a few minutes, raising it step-by-step from the oil and maintaining it in each position for a few minutes, then lowering in the medium to 85 its base end and pouring water into its interior, then heating the base while maintaining the end portion in water, then allowing the shell to cool down and then quenching it outright.

95 3. The process of treating an armor piercing projectile which consists in heating the shell to a hardening temperature, to bring the shoulder to a higher temperature than the point and the point to a higher temperature than the base, then dipping the shell point downward to its base in a cooling medium, maintaining it in that position for a few minutes, raising it about one third of its length more or less and there maintaining it for a few minutes, then raising to about two-thirds of its length more or less and there maintaining for a somewhat longer time, then lowering in the medium to the base end and pouring water into its 100 interior, then heating the base to a substantially lower temperature than the first heating while maintaining the end portion in a cooling medium, then allowing the shell to cool down and then quenching it outright, 105 substantially as described.

110 4. The herein described process of hardening an armor piercing projectile which consists in a double treatment substantially as follows, first heating the external shoulder 115 of the shell to about 920° to 930°, more or less, the inner surface adjacent the shoulder to about 900°, more or less, the point to a temperature of about 875° to 880°, more or less, and the base to a temperature substantially lower, then dipping the shell in oil to its base and maintaining it in that position about eight to fourteen minutes, more

- or less, then raising the shell in the oil about one-third of its length and maintaining it in that position for rather more than eight minutes more or less, then raising it 5 to a zone depth of about one-third of its length, more or less, and maintaining it in that position for a longer time, then lowering the shell into the oil to its base and pouring water into its interior, then 10 reheating the shell base to about 650° to 725°, more or less, and its core to about 600° to 650° more or less, while its point is immersed in water to rather less than one-third the shell length, then permitting the 15 shell to cool to a temperature of from about 250° to about 350° more or less, and then quenching outright in water.
5. The process of treating an armor piercing projectile which consists in heating the 20 shell to bring the shoulder to a higher temperature than the point, dipping the shell point downward in a cooling medium, raising it partially from said medium, then dipping again into the medium.
6. The process of treating an armor piercing projectile which consists in heating the 25 shell to a hardening temperature, protecting the point and bringing the shoulder to a higher temperature than the point, then immersing the shell, point down, in a cooling 30 medium, raising the shell but leaving

a portion in said medium, then lowering the shell into the medium.

7. The process of treating an armor piercing projectile which consists in heating the 35 shell to a hardening temperature, while protecting the point to bring the shoulder to a higher temperature than the point and the point to a higher temperature than the base, then dipping the shell point downward in 40 a cooling medium, raising the shell in the medium step by step to a plurality of positions and maintaining the shell a short time in each of said positions.

8. The process of treating an armor piercing projectile which consists in applying a protector to the point so as to protect the point from direct contact with the heat, then heating the shell in a furnace to bring the shoulder to a higher temperature than 50 the point, then dipping the shell in a cooling medium, point downward, partially raising the shell from the medium, then lowering the shell into the medium.

Signed at London, England, this sixth 55 day of August 1913.

ROBERT ABBOTT HADFIELD.

ALEXANDER G. M. JACK.  
ISAAC BERNARD MILNE.

Witnesses:

ARTHUR WOODNAM,  
CHARLES VIVIAN GURNEY.